

Dec. 1, 1959

**R. L. YAMARTINO**

**2,915,383**

## METHOD OF PRODUCING REFRACTORY METALS

Filed Jan. 3, 1955



INVENTOR.  
Raymond L. Yamartino  
BY  
Oliver W. Hayes

1

2,915,383

## METHOD OF PRODUCING REFRactory METALS

Raymond L. Yamartino, Waltham, Mass., assignor to National Research Corporation, Cambridge, Mass., a corporation of Massachusetts

Application January 3, 1955, Serial No. 479,483

4 Claims. (Cl. 75—84.5)

This invention relates to the production of metals and more particularly to the production of refractory metals such as titanium and the like. In the previous application of Keller et al., Serial No. 434,648, filed June 4, 1954, now Patent No. 2,846,304, granted August 5, 1958, there is described a process for the production of titanium in which high yields of large crystals of titanium are obtained by the two-stage reduction of a titanium halide. It is a principal object of the present invention to provide an improved apparatus and process particularly adapted for utilization with the invention described in the above Keller et al. application.

Another object of the invention is to provide an improved process for localizing the production of refractory metal crystals.

Still another object of the invention is to provide an improved apparatus for operation of a process of the above type.

Other objects of the invention will in part be obvious and will in part appear hereinafter.

The invention accordingly comprises the process involving the several steps and the relation and the order of one or more of such steps with respect to each of the others, and the apparatus possessing the construction, combination of elements and arrangement of parts which are exemplified in the following detailed disclosure, and the scope of the application of which will be indicated in the claims.

For a fuller understanding of the nature and objects of the invention, reference should be had to the following detailed description taken in connection with the accompanying drawing.

In the present invention, the refractory metal compound is dissolved in a fused salt and is reduced to the refractory metal in the form of relatively large crystals by means of a liquid metal reducing agent. In a preferred embodiment of the invention, the refractory metal compound is a titanium halide so that titanium crystals are the end product. The present invention also preferably includes a two-stage reduction of the titanium halide to first produce a solution of titanium lower halides in a fused salt such as sodium chloride. The titanium halide dissolved in the molten salt is then preferably reduced to metallic titanium by means of a reducing agent which is sprayed across the surface of the solution. This reducing agent is preferably sodium, and the invention will be described in connection with the utilization of sodium as the reducing agent, titanium lower chlorides as the titanium halide, and sodium chloride as the fused salt.

The present invention is particularly directed to improvements in apparatus and techniques for accomplishing the second stage reduction. As pointed out in the Keller et al. application Serial No. 434,648, it is highly desirable to so conduct the second stage reduction that sodium is uniformly sprayed across the surface of a solution of titanium dichloride in fused sodium chloride. As a result of this spraying, a crust of fine particles of

2

titanium forms at the surface of the fused salt. This crust has some mechanical strength due to the sintering of the fine titanium particles to each other, but the crust is preferably supported every few inches or so by means of a suitable grid or the like, this grid being helpful in preventing collapse of the crust in later stages of the titanium crystal growth. As more sodium is fed to the salt bath, the level of the salt tends to rise above the crust due to the formation of more sodium chloride. During this further feed of sodium, titanium crystals grow from the bottom of the crust to form an interlaced mass of relatively large titanium crystals, many of which have dimensions on the order of an inch or so. When it is desired to remove the product titanium from the reactor, it has been found that, in many cases, some of the titanium is quite firmly fastened to the walls of the reactor. It is necessary to chip this titanium from these walls, a fairly time-consuming and relatively expensive operation. In the present invention, adhesion of the product titanium to the reactor wall is substantially prevented by isolating and localizing the titanium crystal growth. This is accomplished in a preferred embodiment by feeding the sodium to a limited portion of the bath containing the dissolved dichloride and isolating this limited portion of the bath, particularly at the surface, from the remainder of the bath. The space above the limited portion is also preferably isolated from the space above the remainder of the bath so as to prevent migration of sodium vapors from the point of feed to the other portions of the bath. Additionally, the means for isolating the point of sodium feed from the remainder of the bath is electrically insulated from the main walls of the reaction chamber. Accordingly, any flow of electrons from the point of sodium feed to the point of minimum sodium concentration adjacent the reactor walls is substantially prevented.

Referring now to the drawing, there is illustrated one method of practicing the invention wherein 10 represents a reactor containing a charge of fused salt 12, this fused salt preferably comprising sodium chloride and containing a dissolved mixture of titanium dichloride and titanium trichloride. Positioned within the fused salt is a cylinder 13, this cylinder 13 preferably comprising nickel, titanium or the like and extending upwardly into space 14 above the fused salt 12. The upper end of cylinder 13 is supported by a flange 15 so that space 14a above the interior of the cylinder 13 is isolated from the remainder of the space 14. The reactor also includes a cover 16, a plurality of insulating gaskets 18, and clamps 20 for holding the cover on the reactor 10 and also for positioning the cylinder 13. Sodium is preferably fed through a pipe 21 to the space 14a, being distributed by means of a spinning disc 22 of the type described in the copending application of Hellier, Serial No. 442,525, filed July 12, 1954, now abandoned. If desired, titanium crust supports 23 may be provided within cylinder 13.

The pressure in the space 14a is preferably maintained equal to that in the space 14, although the pressure-equalizing means is so arranged as to prevent transfer of sodium vapors from the space 14a to space 14. This pressure-equalizing means, in a preferred embodiment, comprises a tube 24, a sodium condenser 26, and another tube 28. Through this tube 28 an inert gas pressure of equal magnitude can be applied to each of the two spaces, 14 and 14a respectively, by means of a valve 30 and an inert gas supply 32.

In the operation of the device illustrated in the drawing, a charge of titanium dichloride dissolved in molten sodium chloride is provided in reactor 10, preferably after all air has been removed therefrom. This molten salt may be fed to the reactor through a suitable open-

ing (not shown). Sodium is then fed at a relatively slow rate, for example, on the order of 2 pounds per hour per square foot of molten sodium chloride surface. The sodium is preferably sprayed uniformly across the surface of the salt bath inside of cylinder 13 so as to initially form a titanium crust, as described in the above mentioned Keller et al. application Serial No. 434,648, this crust being supported by supports 23. Further feed of sodium provides for dissolution of sodium in a layer of relatively pure sodium chloride which is localized by the crust. Simultaneously, titanium crystals commence growing from the underside of the titanium crust and from both sides of cylinder 13. Since cylinder 13 is electrically insulated from the reactor walls, electrons do not travel to the wall 10 and titanium crystal growth will not start outwardly from the reactor walls. Accordingly, titanium crystal growth is localized on the cylinder 13. When the reaction has been substantially completed, cylinder 13 can be removed from the residual salt, carrying therewith a mass of titanium crystals adhering thereto. If desired, additional supports for the titanium crystals can be provided on the interior and exterior surfaces of cylinder 13. Additionally, holes may be provided in cylinder 13, below the surface of the bath, to assist in providing return paths for the chloride ions.

While only one cylinder 13 has been shown, numerous other cylinders may be provided. Equally, many shapes other than cylinders may be employed for isolating the limited portions to which sodium is fed. Additionally, other types of insulation may be provided on the insulating gaskets 18 illustrated. Frozen salt may be employed or ceramics when the temperature is such that reaction between the insulator and the sodium or other vapors is not a problem. If desired, a titanium crust breaker of the type described in the copending application of Vaughan, Serial No. 478,652, filed December 30, 1954, can be employed. Equally, feed of sodium below the surface can be accomplished as described in the copending application of Keller et al., Serial No. 470,453, filed November 22, 1954, now Patent No. 2,848,319, granted August 19, 1958.

While the invention has been described in a modification wherein equal pressures are provided in the spaces 14 and 14a, it should be apparent that a predetermined difference in pressure may be maintained in these two spaces. Thus one space may have a higher inert gas pressure than the other space. Many other means of equalizing these pressures can also be employed.

Numerous alternative methods of practicing the present invention may be employed. For example, the temperature of the reaction mass may be widely varied from slightly above the melting point of the salt to temperatures on the order of 1000° C. and above. Numerous reducing agents other than the sodium can be employed, for example, potassium, calcium, magnesium, lithium and various combinations of these elements may be utilized. From the standpoint of cheapness, sodium, sodium-potassium alloy or magnesium are preferred.

Other halides of titanium may be utilized, although, from the standpoint of cost, ease of handling, etc., the tetrachloride is preferred.

Additionally, the reactor can be fed with lower halides of titanium such as titanium trichloride manufactured from titanium-bearing materials in the manner shown in the copending applications of Singleton, Serial No. 304-388, filed August 14, 1952, now Patent No. 2,770,541, granted November 13, 1956, and Singleton, Serial No. 315,461, filed October 18, 1952, now abandoned. Equally, titanium trichloride can be made by the technique described by Sherfey et al., Journal of Research of the Bureau of Standards, 46, 299-300, April 1951. Additionally, the dichloride of titanium can be manufactured by numerous processes such as disproportionation of the trichloride or partial reduction of the trichloride or tetrachloride.

The present invention can be equally employed for the manufacture of titanium alloys by the coreduction of the chlorides, for example, of zirconium, vanadium, chromium, manganese, iron, nickel, cobalt, columbium, tantalum, molybdenum, tungsten or silicon. The alloy may be a binary alloy or it may be an alloy containing three or four constituents. In the manufacture of alloys, the same general conditions of the reduction of the titanium halide and reducible compounds of the alloying constituents must be employed. Accordingly, when used in the claims, the word "titanium" is intended to mean alloys thereof as well as the pure metal.

While the invention has been particularly described in connection with the production of titanium, it is also applicable to the production of other refractory metals such as zirconium, thorium, vanadium, columbium, tungsten, tantalum, molybdenum and the like by the reduction of reducible compounds such as the halides of such refractory metals dissolved in suitable fused salts. It should be additionally pointed out that the salt mixture in which the reduction is carried out may be formed of numerous halides which can be mixed halides, single halides and halides of materials other than the specific reducing agent or agents employed in the reaction. From the standpoint of simplicity of operation and ease of control, however, it is preferred that the salt be the chloride of the reducing agent. It is quite feasible to employ binary and ternary mixtures of halides having quite low melting points.

It should be pointed out, in connection with a consideration of the various salts which can be employed, that these salts should be completely anhydrous and free of any contaminants such as carbon, nitrogen, oxygen or hydrogen. This is particularly true when making metals such as titanium due to the tremendous reactivity of titanium metal at temperatures on the order of 800° C. to 900° C. and above.

In the above specification, reference has been made particularly to the preferred titanium chlorides, tetrachloride and dichloride. In most instances, the trichloride is equally useful and, as a matter of fact, it is extremely unlikely that any system having an appreciable concentration of one of the lower chlorides of titanium will not have at least some of the other lower chloride also present. It should be apparent that one can also employ the corresponding di-, tri-, and tetrahalides from the group consisting of the iodides, bromides and fluorides of titanium.

Since certain changes may be made in the above process and apparatus without departing from the scope of the invention herein involved, it is intended that all matter contained in the above description, or shown in the accompanying drawing, shall be interpreted as illustrative and not in a limiting sense.

What is claimed is:

1. In a process for manufacturing a refractory metal selected from the group consisting of zirconium, thorium, vanadium, columbium, tungsten, tantalum, and molybdenum where a halide of the refractory metal dissolved in a molten salt is reduced to refractory metal by means of a liquid metal reducing agent selected from the class consisting of lithium, sodium, potassium, magnesium and calcium and mixtures thereof, the molten salt comprising at least one halide selected from the class consisting of the alkali metal halides and the alkaline earth metal halides, the improvement which comprises confining the fused salt bath in a metal-walled reactor, adding molten reducing agent to a limited portion of the fused salt bath, preventing passage of reducing vapors from the limited portion to the space above the remainder of the bath by means of a vapor barrier, equalizing the gas pressures existing above the limited portion and the remainder of the bath, and electrically insulating the metal reaction chamber walls from the vapor herein.
2. In a process for producing titanium wherein a lower

halide of titanium is dissolved in a fused salt bath and is reduced to titanium crystals by means of a metallic reducing agent selected from the class consisting of the alkali metals and the alkaline earth metals, the molten salt comprising halide selected from the group consisting of the alkali metal halides and the alkaline earth metal halides, the improvement which comprises confining the fused salt bath in a metal-walled reactor, adding molten reducing agent to a limited portion of the fused salt bath, preventing passage of reducing agent vapors from the limited portion to the space above the remainder of the bath by means of a vapor barrier, equalizing the gas pressures existing above the limited portion and the remainder of the bath, and electrically insulating the metal reaction chamber walls from the vapor barrier.

3. In a process for producing titanium wherein a lower halide of titanium is dissolved in a fused salt bath and is reduced to titanium crystals by means of a metallic reducing agent selected from the class consisting of the alkali metals and the alkaline earth metals, the molten salt comprising a halide selected from the group consisting of the alkali metal halides and the alkaline earth metal halides, the improvement which comprises confining the fused salt bath in a metal-walled reactor, adding molten reducing agent to a limited portion of the fused

5

10

15

20

25

salt bath, preventing passage of reducing agent vapors from the limited portion to the space above the remainder of the bath by means of a vapor barrier, and electrically insulating the metal reaction chamber walls from the vapor barrier.

4. The process of claim 2 wherein the titanium lower halide is a titanium lower chloride and the reducing agent comprises sodium.

#### References Cited in the file of this patent

##### UNITED STATES PATENTS

|           |             |               |
|-----------|-------------|---------------|
| 452,030   | Castner     | May 12, 1891  |
| 2,478,594 | Queneau     | Aug. 9, 1949  |
| 2,586,134 | Winter      | Feb. 19, 1952 |
| 2,607,674 | Winter      | Aug. 19, 1952 |
| 2,621,121 | Winter      | Dec. 9, 1952  |
| 2,647,826 | Jordan      | Aug. 4, 1953  |
| 2,739,115 | Gall et al. | Mar. 20, 1956 |
| 2,783,192 | Dean        | Feb. 26, 1957 |

##### OTHER REFERENCES

Handbook of Chemistry and Physics, 26th edition, 1942, pages 402, 403, 450, 451, 476 and 477.  
Journal of Metals, April 1950, pages 634-640.